

Feb. 14, 1956

J. G. CALTON

2,734,794

PROCESS FOR WET-DRAWING POLYETHYLENE TEREPHTHALATE

Filed July 12, 1951



INVENTOR.  
Joseph Gordon Calton  
BY

*Norma E. Buckman*  
ATTORNEY.

1

2,734,794

**PROCESS FOR WET-DRAWING POLYETHYLENE TEREPHTHALATE**

Joseph Gordon Calton, Buffalo, N. Y., assignor to E. I. du Pont de Nemours and Company, Wilmington, Del., a corporation of Delaware

Application July 12, 1951, Serial No. 236,399

5 Claims. (Cl. 18—54)

This invention relates to a process for preparing resilient polyethylene terephthalate fibers and is particularly concerned with a process for producing polyethylene terephthalate fibers and yarn possessing desirable characteristics of fine wool.

Considerable research effort has been directed toward discovering or developing a satisfactory substitute for natural wool. A particular aim has been to produce a synthetic fiber possessing the desirable characteristics of fine wool, such as that used in suits and outer garments, in addition to launderability and freedom from attack by moths. Various synthetic fibers have been subjected to many different processes, both mechanical and chemical, in an effort to so modify their properties that they could be classified as wool-like material. The prior art discusses at length the use of stable fiber-making equipment and crimpers, as well as various chemical and heat-treating methods, for treating synthetic fibers in order to secure characteristics normally associated with natural wool. In no instance, however, have these synthetic materials been satisfactory substitutes for wool. Other than in superficial appearance, they cannot properly be classified as wool-like. A great new field of use would be open to a synthetic fiber which could be woven into fabrics having the hand, resilience, wrinkle-resistance, fullness, warmth, and other such properties normally associated with fine woolen fabrics.

It has now been found that desirable wool-like characteristics can be built into fibers and yarns prepared from the new synthetic linear polyesters described in United States Patent No. 2,465,319 to Whinfield and Dickson. These are highly polymeric linear esters of terephthalic acid which are high melting, difficultly soluble, substantially colorless materials suitable for forming into filaments. The filaments can be extended by drawing into strong flexible fibers showing, by characteristic X-ray patterns, molecular orientation along the fiber axes. This has been accomplished by drawing the fibers at elevated temperatures to a high draw ratio, i. e., to several times the original fiber length.

It is an object of this invention to provide a process for producing polyethylene terephthalate fibers having the resilience characteristics of the better grades of wool. A further object is to provide a process for preparing uniform, drawn polyethylene terephthalate fibers of wool-like properties, which fibers will not be subject to additional cold drawing during subsequent normal processing. Other objects will become apparent from the following description of the invention and the appended claims.

These objects are accomplished by drawing polyethylene terephthalate fibers which have a birefringence in the range of 0.004 to 0.11 to 90% to 100% of the maximum draw ratio obtainable at temperatures in the range of 35° to 50° C. while the fibers are wet with a hydroxylated non-solvent, preferably water or a dilute aqueous solution.

With wet fibers having the specified birefringence the

2

maximum draw ratio obtainable at 35° to 50° C. will be within the range of about 2.7 to 4.1 times. The resilient properties associated with fine wools are developed in the drawn polyethylene terephthalate fibers by subsequently relaxing them in a free-to-shrink condition at temperatures in the range of 90° to 200° C.

In the accompanying drawing the single figure illustrates schematically a front elevation of a form of apparatus for drawing yarn in accordance with the above process.

The above process conditions are critical, as will be set forth in greater detail subsequently. However, it may be emphasized at this point that the desired properties will not be obtained unless the fibers are subjected to at least 90% of the maximum draw and the maximum draw ratio is from about 2.7 to 4.1 times the original length of the fibers. It had previously been thought that polyethylene terephthalate fibers must be drawn at temperatures of 60° C. and above in order to avoid excessive breaking of the filaments during the process. However, the maximum draw at 60° C. greatly exceeds 4 times. When an attempt is made to use partial draw ratios as low as 3 to 4 times at temperatures of 60° C. or above, even in the presence of water, the process is extremely difficult to control and the product is not uniform. Such partial drawing at temperatures of 60° C. and above gives rise to non-uniformities of dye receptivity, non-uniformities of denier, and the product undergoes further cold-draw at relative low tension levels during subsequent mill-processing, particularly in staple spinning operations.

Certain conditions referred to above or elsewhere in the specification require explanation. The fiber-forming material is principally polyethylene terephthalate but the inclusion therein of up to 10 mol per cent of modifying material is intended whenever the expression polyethylene terephthalate material is used. Polyethylene terephthalate, itself, is a poly-condensation product of ethylene glycol and terephthalic acid or an ester-forming derivative thereof. During the preparation of this polyester, minor amounts of a modifying material may be added, for example, another glycol and/or another dicarboxylic acid. Thus a suitable funicular structure comprised essentially of polyethylene terephthalate may have included in the polymer molecule up to 10 mol per cent of another glycol such as diethylene glycol, tetramethylene glycol or hexamethylene glycol. Or again, the molecule may contain up to 10 mol per cent of another acid. As suitable examples of modifying acids, there may be mentioned hexahydroterephthalic acid, bibenzoic acid, adipic acid, sebatic acid, azelaic acid, the naphthalic acids, 2,5-dimethylterephthalic acid and bis-p-carboxyphenoxyethane.

These modifiers may be added as one of the initial reactants during the polymerization process, but the modifying materials may also be polymerized separately and then melt-blended with the polyethylene terephthalate. In either case, the total amount of modifier in the final polymeric material should not exceed 10 mol per cent. The polyesters are suitably prepared as described in U. S. Patent 2,465,319.

The ethylene terephthalate polymer preferably has an intrinsic viscosity of at least 0.3. Those polymers having lower intrinsic viscosities are essentially non-fiber forming. The expression "intrinsic viscosity" is used herein as a measure of the degree of polymerization of the polyester and may be defined as

$$\text{limit } \frac{\ln (r)}{C}, \text{ as } C \text{ approaches } 0$$

70 wherein  $r$  is the viscosity of a dilute solution of the polyester in a mixture of 60 parts phenol and 40 parts tetra-

chloroethane, divided by the viscosity of the phenol-tetra-chloroethane mixture, per se, measured in the same units at the same temperature, and C is the concentration in grams of polyester per 100 cc. of solution.

The yarns and fibers prepared in accordance with the process of this invention possess a property of wool which is most difficult to duplicate, namely, resilience. This property is not easy to measure quantitatively, but may be defined to a considerable extent by three important parameters: Initial tensile modulus, tensile recovery, and compliance ratio.

The "initial tensile modulus" (represented by the symbol  $M_i$ ) is defined as the slope of the first reasonably straight portion of a stress-strain curve of the funicular structure obtained by plotting tension on a vertical axis vs. elongation on a horizontal axis as the structure is being elongated at the rate of 10% per minute under standard conditions of temperature (21° C.) and humidity (60% RH). In almost every instance, this first reasonably straight portion is also the steepest slope to be found on the curve. The values as used herein are in units of kilograms per square millimeter per 100% elongation.

The initial tensile modulus,  $M_i$  is a measure of resistance to stretching and bending. The effects of the filament modulus are felt in a fabric chiefly when the fabric is folded or crushed in the hand or otherwise handled. If the modulus is too low, the fabric is "rubbery" or "limp"; with too high a modulus in the fibers, the fabric is "wiry" or "boardy." When the modulus is in the proper range, a "soft" fabric results. Attempts have been made to counteract the effects of a modulus lying outside the wool range by a suitable adjustment of filament diameter. In each instance, this straying away from the usual diameters of wool filaments has resulted in deleterious effects on properties such as liveliness and recovery from wrinkling. Since the filament properties which are almost entirely responsible for fabric resistance to bending are (1) the initial modulus and (2) the diameter, and since the range of suitable diameters seems to be confined to those typical of wool, it follows that a wool-like handle will be obtained in the fabric when fibers having an initial modulus in the wool range are used.

The "tensile recovery" (TR) is defined as the extent to which the yarn recovers its original length after being stretched, a stress-strain curve being used to determine tensile recovery under the testing conditions. The test consists in extending the funicular structure at a constant rate of elongation of 10% per minute. A specimen is held at the maximum elongation desired for 30 seconds, e. g., by the use of a time switch, and is then allowed to retract at the same rate at which it was extended. The same specimen is extended approximately 1.0, 3.0 and 5.0% for each determination. The extension during elongation and the recovery during retraction are measured along the elongation axis. The tensile recovery is then the ratio of the extent to which the yarn retracts to the extent to which it was elongated. This test is run under standard conditions at 60% RH and 21° C.

It is well known that resistance to wrinkling and massing and rapid recovery from unavoidable wrinkles are highly desirable traits in apparel fabrics. The tensile recovery correlates in a high degree with these properties. The tensile recovery from a 1% elongation correlates with fabric recovery from mild wrinkling, and, as might be expected, the tensile recovery from higher elongations correlates with recovery from more severe wrinkling and sharp creasing. In this instance, the words, "resistance to" may be used alternatively to "recovery from" since resistance to a crease or wrinkle really involves a very rapid and complete recovery from a crease or wrinkle when the deforming force is removed. The rapid recovery is a characteristic of the polyethylene terephthalate materials of this invention.

The "compliance ratio" (CR) is associated with the shape of a stress-strain curve and is a measure of the

rate of change of compliance with elongation. Compliance is defined as elongation divided by tension in kg./mm.<sup>2</sup>. Hookean systems, those for which the stress-strain curve is a straight line, exhibit equal compliance at all elongations, and for these the change of compliance with elongation is 0. On the other hand, one of the most important properties of wool is its change toward higher compliance as it is progressively deformed. It is this property which enables wool to feel simultaneously crisp and soft. This property is measured by determining the average rate at which compliance changes in the range 5 to 10% elongation and is computed by the following formula:

$$CR = \frac{1}{5} \left( \frac{10}{\text{Tension at 10\% elongation}} - \frac{5}{\text{Tension at 5\% elongation}} \right)$$

The stress-strain curve of wool has two distinctly different regions, consisting of (1) an initial portion in which the resistance to deformation is relatively great, and (2) 20 a later portion in which the resistance decreases regularly and to a high degree. It is for this reason that a wool fabric which is crisp and firm to the touch will feel soft and compliant when severely crushed in the hand. Among the natural fibers this dualistic behavior is found 25 only in wool and other animal hairs (not in silk, cotton, etc.), and this is one of the most attractive and valuable characteristics of wool.

In applying the above methods for evaluating wool-like resilience, it has been found that the better grades of wool 30 for outer garment uses have values for these three parameters in the following ranges:

$$Mi = 110 \text{ to } 550 \text{ kg./mm.}^2$$

$$CR = 0.05 \text{ to } 0.17$$

$$TR = 55\% \text{ or more from extensions of } 3\%$$

In accordance with the process of the present invention synthetic yarns or fibers are produced which have wool-like resilience within the above limits. Furthermore, the resulting synthetic fibers have these desirable resilience 40 characteristics throughout by virtue of uniform treatment therealong during formation and subsequent processing.

The following examples are illustrative of this invention and are not to be construed as limitative. The birefringence (or double refraction) of the filaments was measured by the retardation technique described in "Modern Textile Microscopy" by J. M. Preston (London, 1933) page 270, using a petrographic microscope (Bausch & Lomb, Model LB) together with a Bausch & Lomb style B cap analyzer compensator.

#### EXAMPLE 1

Polyethylene terephthalate in chip form having an intrinsic viscosity of 0.60 was melted on a heated grid and metered through a suitable filter pack. It was then 55 extruded through a spinneret having fifty-three holes into room temperature air. The extruded filaments were cooled and solidified by passage through the air and subjected after solidification to a means for winding them into a suitable package at the rate of 1206 yards per minute. The filaments of this 460 denier yarn exhibited a birefringence of 0.0060.

Several ends of yarn prepared in this fashion were combined to form a tow which was metered by a series of four rolls, each comprising at a surface speed of 52 yards 60 per minute, into an aqueous bath heated to a temperature of 40° C. and containing 1.4% by weight of Avitex R, a fatty alcohol sulfate textile finishing agent. The tow was withdrawn from the bath by means of a series of four rolls, each operating at the speed of 52 yards per minute, and each roll being heated to 40° C. The tow was then passed to a series of unheated draw rolls, operating at peripheral speeds of 200 yards per minute, thereby drawing the tow to about 3.85 times its previous length. From the draw rolls, the tow was passed through 70 a stuffing box type crimper, operating to apply 10-12

crimps per inch. The tow was then dropped in a free-to-shrink condition onto an endless belt which carried it through an air oven heated to 155°-165° C., the period of travel through the oven being two minutes. The resulting relaxed product, before or after cutting into staple, possessed the properties shown in the following table:

Table I

|                                              |       |
|----------------------------------------------|-------|
| Tenacity in grams/denier                     | 3.3   |
| Elongation at break percent                  | 40    |
| Initial modulus in kg./mm. <sup>2</sup>      | 317   |
| Compliance ratio                             | 0.067 |
| Tensile recovery from 3% elongations percent | 55    |

## EXAMPLE 2

Polyethylene terephthalate having an intrinsic viscosity of 0.61 was spun into a yarn in the manner described in Example 1, at a speed of 978 yards per minute. The filaments of this yarn exhibited a birefringence of 0.0058. This yarn was processed into three denier-per-filament staple essentially as described in Example 1. The yarn was drawn about 3.85 times at 40° C., using water to wet the yarn instead of the aqueous finish bath of Example 1. Before cutting to staple the tow was relaxed in a boiling water shower and dried. These staple fibers had the properties shown in Table II.

Table II

|                                              |       |
|----------------------------------------------|-------|
| Tenacity in grams/denier                     | 2.85  |
| Elongation at break percent                  | 62    |
| Initial modulus in kg./mm. <sup>2</sup>      | 249   |
| Compliance ratio                             | 0.103 |
| Tensile recovery from 3% elongations percent | 60    |

## EXAMPLE 3

A copolyester prepared from ethylene glycol and a mixture of terephthalic acid and sebacic acid, containing 95% by weight of terephthalic acid and having an intrinsic viscosity of 0.58, was spun into yarn in the manner of Example 1 at a speed of 978 yards per minute. The filaments of this yarn exhibited a birefringence of 0.0048. This yarn was processed into three denier-per-filament staple in the manner described in Example 1. The properties of the final staple product are listed in Table III.

Table III

|                                              |       |
|----------------------------------------------|-------|
| Tenacity in grams/denier                     | 2.6   |
| Elongation at break percent                  | 51    |
| Initial modulus in kg./mm. <sup>2</sup>      | 280   |
| Compliance ratio                             | 0.089 |
| Tensile recovery from 3% elongations percent | 55    |

## EXAMPLE 4

In two separate experiments, polyethylene terephthalate having an intrinsic viscosity of 0.59 was spun at the speed of 1206 yards per minute into yarn suitable for processing into 1.5 and 4.5 denier-per-filament staple respectively. Filaments from the heavier denier-per-filament yarn exhibited a birefringence of 0.0072, while those from the finer denier yarn had a birefringence of 0.0085. Both of these yarns were processed into staple by the technique described in Example 1. The properties of the staple fibers are shown in Table IV.

Table IV

|                                              | 1.5 denier | 4.5 denier |
|----------------------------------------------|------------|------------|
| Tenacity g/d                                 | 3.5        | 3.5        |
| Elongation percent                           | 45         | 40         |
| Initial modulus                              | 300        | 305        |
| Compliance ratio                             | 0.075      | 0.068      |
| Tensile recovery from 3% elongations percent | 60         | 55         |

The filaments from polyethylene terephthalate yarn exhibiting a birefringence outside the range of 0.004 to 0.011 will not draw satisfactorily according to the process

of this invention. When the birefringence is less than 0.004, one encounters excessive breakage and undrawn filaments in attempting to draw at temperatures below 60° C. On the other hand, when the filaments exhibit a birefringence above 0.011, they cannot be drawn 2.7 to 4.1 times at 35°-50° C., and the desired resilient product is not obtained with lower draw ratios. While they can be drawn at higher temperatures, the initial modulus of the drawn product is then considerably higher than that of fine wool.

When as-spun polyethylene terephthalate filaments exhibit birefringence in the critical range from 0.004 to 0.011 the polymer molecules are not distributed randomly, but in some regular manner. It is perhaps the beginning of orientation, although orientation does not show up in X-ray diagrams of the material.

The birefringence of the polyethylene terephthalate as-spun filaments is dependent upon the polymer intrinsic viscosity, the spinning speed and the rate of cooling of the freshly spun filaments. All other conditions being equal, an increase in the polymer intrinsic viscosity results in a corresponding increase in the birefringence exhibited by the filaments. The birefringence also increases with spinning speed as measured at the take-up and with more rapid cooling of the filaments as they leave the spinneret. This is illustrated to some extent in Example 4, where the heavier denier filaments, which do not cool as fast as the finer denier filaments, exhibits a lower birefringence.

The polyethylene terephthalate multi-filament yarn used in the process of this invention for the preparation of textile denier filament yarn and staple is readily prepared by spinning 0.50 to 0.70 intrinsic viscosity polymer at speeds in the range of about 900 to 1800 yards per minute. Of course, higher viscosity polymer can be used at lower spinning speeds, but such a process is not as economical. On the other hand, lower intrinsic viscosity polymers can be spun at higher speeds to obtain the proper birefringence. However, the spinning of the lower molecular weight polymers is more difficult and the tensile properties of the yarn are not so good as those of the higher intrinsic viscosity polymer yarn. Surprisingly, the polyethylene terephthalate yarn spun in the preferred manner differs from that described in the prior art, in that it can be stored indefinitely before drawing without becoming brittle and difficult to process.

The yarn should be drawn to at least 90% of its maximum extensibility at 35° to 50° C., a draw ratio of nearly 4.1 times generally being obtained, although the ratio may be as low as 2.7 times with some yarns of the class described, particularly those whose birefringence is at or near 0.011. At temperatures below 35° C., the desired draw ratio is difficult to obtain and the physical properties of the final yarn are below the desired level. At temperatures much above 50° C., the maximum draw ratio rapidly increases and yarn drawn to 90%-100% of the maximum extensibility will not possess the resilient properties of fine wool. If the yarn is only partially drawn to a draw ratio of 4 at temperatures above 50° C., both denier and dyeing non-uniformity result.

The yarn should be wet thoroughly before passing over the draw rolls. Any hydroxylated non-solvent may be used, such as water, ethylene glycol, glycerol, and the like. Water and dilute aqueous solutions containing a finish for the yarn are preferred. As illustrated in Example 1, it is quite convenient to apply the yarn finish at this point in the process. The yarn may be wet by any conventional means.

The schematic apparatus shown in the accompanying drawing represents a convenient method for wetting and drawing the yarn. In this figure, the tray 13 contains wetting liquor heated to a temperature of around 40° C. The yarn 14 to be drawn is fed over rolls 1, 2, 3 and 4, passes through the liquid bath, and is then fed over rolls 5 through 12, respectively. Rolls 5, 6, 7 and 8 are

heated to the same temperature as the bath. The remainder of the rolls are not heated. Rolls 1 through 8 are rotated at the same peripheral speed while rolls 9 through 12 have a peripheral speed of 2.7 to 4.1 times greater. Neglecting slippage on the rolls, a drawing of 2.7 to 4.1 times takes place between rolls 8 and 9.

The drawing process is applicable to single ends of yarn, to a plurality of yarn ends in warp form, or to heavy denier tows. At the low temperatures involved, heating the yarn uniformly is no problem. Equipment can, therefore, be simple and operational difficulties minimized.

While the fibers and yarn prepared in accordance with this invention are capable of some spontaneous crimping when relaxed, as by being heated to an elevated temperature under little or no tension, it is preferred to crimp them mechanically. This can be accomplished conveniently by passing a tow comprising several ends of yarn through a stuffing box type crimper. The crimping operation is not essential in providing the final yarn with the resilience properties of fine wool, but it aids in subsequent mill processing. If the yarn is to be mechanically crimped, this operation is performed preferably after drawing and before relaxation.

The yarn finally acquires the resilience properties of fine wool during relaxation and setting. The yarns are relaxed and set by heating them to temperatures in the range of 90° to 200° C. under little or no tension. Suitable heating media include hot air, hot or boiling water, saturated or super-heated steam and various hot solutions that exert a mild plasticizing action on the material, for example, dilute nitric acid. At the higher temperatures, for example, around 150° C., the treatment may be for short periods of time, such as two minutes. Treatment at the lower temperatures should generally be for longer periods of time ranging up to 15 minutes or more, although exposure of the fibers to a shower of water at 90°-100° C. for a few seconds has been used successfully. This heat treatment stabilizes the yarn and increases the degree of crystallization, and also reduces residual shrinkage at the same time. If desired, the fibers may be forwarded directly from the drawing operation, or after crimping, through a suitable bath or heated chambers before being wound up or cut into staple.

Prior to this invention, textile-denier filaments of polyethylene terephthalate could not be drawn at temperatures below 60° C. without excessive breakage, even when wet. The as-spun yarn was known to become brittle on standing, and subsequent drawing of the brittle yarn was difficult even at temperatures above 60° C. The discovery that filaments of polyethylene terephthalate having a birefringence of 0.004 to 0.011 can be drawn wet at temperatures below 60° C. is essential to this process for preparing a synthetic fiber possessing the desirable characteristics of fine wool. Since these filaments do not become brittle on standing, an added advantage is that the as-spun yarn does not have to be drawn soon after spinning.

An outstanding feature of this invention is the production of a uniformly drawn product. The process provides for a means of obtaining a low draw ratio while drawing the yarn to at least 90% of its maximum extensibility. That good denier uniformity is obtained is confirmed by the uniformity of subsequently dyed fabrics. Another important advantage obtained from drawing the yarn to a maximum is that the yarn or staple is substantially free of subsequent cold drawing during mill processing.

The particular fibers prepared by the process of this invention not only duplicate fine wool fibers in appearance, but also duplicate fine wool in the important physical characteristics of initial tensile modulus, tensile recovery and compliance ratio. As a result, a wool-like fabric may be produced from them which is crisp and firm to the touch and, nevertheless, feels soft and com-

pliant when severely crushed in the hand. These fibers and yarns of polyethylene terephthalate materials possess, in addition, much greater strength and wear resistance than wool fibers and are not attacked by moths.

Fabrics made from these fibers are extremely lively and wrinkle resistant, with desirable drape and excellent crease retentivity. They are remarkably insensitive to water and changes in humidity. Also of importance is the versatility which the fibers possess over and above that of wool for processing into fabrics. They are useful, particularly in staple form, in felts of various kinds, including paper-maker's felts, carpets, men's and women's suits, bathing suits, sweaters, knitting yarns, as the warp in Turkish towels and the like.

Suiting fabrics prepared from the staple fibers produced in accordance with this invention are particularly outstanding. These are equal to or better than high grade woolen suiting fabrics in wrinkle resistance, recovery from wrinkling, and retention of ironed creases. Trousers may be cleaned by washing in an automatic washer and hanging them up to dry; they do not shrink appreciably, retain their original creases, and need no further pressing.

Since many different embodiments of the invention may be made without departing from the spirit and scope thereof, it is to be understood that the invention is not limited by the specific illustration except to the extent defined in the following claims.

What is claimed is:

1. In the process for wet-drawing polyethylene terephthalate fibers to obtain strong, molecularly oriented textile fibers the improvement for producing uniform artificial fibers having the resilience characteristics of the better grades of wool which comprises drawing while wet with inert aqueous medium at temperatures in the range of 35° to 50° C. polyethylene terephthalate fibers of textile denier, having a birefringence in the range of 0.004 to 0.011 and a corresponding maximum draw ratio of 4.1 to 2.7 at 35° to 50° C., to at least 90% of said maximum draw ratio and heating the drawn fibers in a free-to-shrink condition at temperatures in the range of 90° to 200° C. until relaxed and set.

2. A process for producing uniform artificial fibers having the resilience characteristics of the better grades of wool which comprises wetting with water polyethylene terephthalate fibers of textile denier having a birefringence in the range of 0.004 to 0.011 and a corresponding maximum draw ratio of 4.1 to 2.7 at 35° to 50° C., drawing the wet fibers at temperatures in the range of 35° to 50° C. to at least 90% of said maximum draw ratio, and heating the drawn fibers in a free-to-shrink condition at temperatures in the range of 90° to 200° C. until wool-like fibers are produced and relaxed and set.

3. A process for producing uniform artificial fibers having the resilience characteristics of the better grades of wool which comprises continuously passing polyethylene terephthalate yarn composed of textile-denier fibers having a birefringence in the range of 0.004 to 0.011 through an aqueous bath which is both non-reactive with and a non-solvent for said fibers, continuously withdrawing the wet yarn from the bath, passing the yarn over heated rolls until the wet yarn is at a temperature of 35° to 50° C., continuously drawing the wet yarn at 35° to 50° C. to a maximum draw ratio of 2.7 to 4.1 times, and continuously passing the drawn yarn through a heating medium at 90° to 200° C. in a free-to-shrink condition until the yarn is relaxed and set and characterized by an initial tensile modulus in the range of 110 to 550 kg./mm.<sup>2</sup>, a compliance ratio in the range of 0.05 to 0.17, and a tensile recovery of at least 55% from extension of 3%.

4. A process for producing uniform artificial fibers having the resilience characteristics of the better grades of wool which comprises preparing polyethylene terephthalate fibers of textile denier exhibiting birefringence

in the range of 0.004 to 0.011 by spinning 0.50 to 0.70 intrinsic viscosity polymer at speeds in the range of about 900 to 1800 yards per minute, wetting the fibers with water, drawing the wet fibers at temperatures in the range of 35° to 50° C. to a maximum draw ratio of 2.7 to 4.1 times, and heating the drawn fibers in a free-to-shrink condition at temperatures in the range of 90° to 200° C. until relaxed and set and characterized by wool-like resilience.

5. A process for producing fibers having the property of relaxing to form uniform fibers having the resilience characteristics of the better grades of wool when heated in a free-to-shrink condition at temperatures in the range of 90° to 200° C. until set which comprises wetting with

5 water polyethylene terephthalate fibers of textile denier having a birefringence in the range of 0.004 to 0.011 and drawing the wet fibers at temperatures in the range of 35° to 50° C. to a maximum draw ratio of 2.7 to 4.1 times.

## References Cited in the file of this patent

## UNITED STATES PATENTS

|    |           |         |       |               |
|----|-----------|---------|-------|---------------|
| 10 | 2,199,411 | Lewis   | ----- | May 7, 1940   |
|    | 2,249,756 | Finzel  | ----- | July 22, 1941 |
|    | 2,285,522 | Alfthan | ----- | June 9, 1942  |

## FOREIGN PATENTS

|         |               |       |               |
|---------|---------------|-------|---------------|
| 603,840 | Great Britain | ----- | June 23, 1948 |
|---------|---------------|-------|---------------|